# EUROPEAN PATENT SPECIFICATION

(11) **EP 2 379 683 B1**
(45) Date of publication and mention of the grant of the patent: **21.06.2017**
(21) Application number: 10700771.8
(22) Date of filing: 08.01.2010
(51) Int. Cl.: C10M 105/38, C10M 107/32, C10M 171/00, C10N 30/02, C10N 30/06, C10N 40/30

(54) **CARBON DIOXIDE-BASED WORKING FLUIDS FOR REFRIGERATION AND AIR CONDITIONING SYSTEMS**
AUF KOHLENSTOFFDIOXID BASIERENDE ARBEITSMEDIEN FÜR KÜHL- UND KLIMATISIERUNGSSYSTEME
FLUIDES DE TRAVAIL À BASE DE DIOXYDE DE CARBONE POUR DES SYSTÈMES DE RÉFRIGÉRATION ET DE CONDITIONNEMENT D'AIR

(30) Priority: 16.01.2009 US 145290 P
(43) Date of publication of application: 26.10.2011
(73) Proprietor: Chemtura Corporation, Middlebury, CT 06749 (US)
(72) Inventor: KELLEY, Richard, Princeton NJ 08540 (US); CARR, Dale, Morristown NJ 07960 (US); HUTTER, Jeffrey, Edison NJ 08817 (US); HESSELL, Edward, Fairfield CT 06825 (US)
(74) Representative: Beacham, Annabel Rose
(86) International application number: PCT/US2010/020453
(87) International publication number: WO 2010/083100

(56) References cited:
- EP-A2- 0 992 572
- WO-A1-2008/105256
- US-A- 5 895 778
- US-A1- 2003 199 401
- US-A1- 2005 127 320
- US-B1- 6 267 907

## Description

### FIELD

This invention relates to carbon dioxide-based working fluids for refrigeration and air conditioning systems.

### BACKGROUND

Carbon dioxide has been used as a working fluid for refrigeration systems as early as at the beginning of modem cryo-engineering. In fact, Linde built the first compression refrigerating machine in 1881 using carbon dioxide as the working fluid. Up to the middle of this century, carbon dioxide was used mainly in ship refrigeration equipment with sub-critical process controls. Glycerine was used as a lubricant. More recently, following the introduction of fluorochlorohydrocarbon refrigerants, carbon dioxide has been largely replaced.

However, carbon dioxide still offers advantages as a working fluid for refrigeration and air conditioning systems, particularly those operating in a trans-critical cyclic process. However, the operating pressures required for such systems are considerably higher than in most present day refrigeration systems. Moreover, in a trans-critical cyclic process, the operating medium is present both in the sub-critical and in the super-critical state, which results in unique lubrication problems. On the one hand, almost complete miscibility between the lubricating oil and CO₂ is required at temperatures as low -40°C. On the other hand, corresponding lubrication and stability properties need to be guaranteed under the influence of CO₂ at pressures of up to 150 bar (15 MPa) and temperatures of up to 220°C. In air conditioning equipment, in particular, the lubricating oil is subject to extreme mechanical and thermal stresses. Tribological difficulties occur in test compressors of the most varied types of design.

In the tribological contact areas subject to the influence of CO₂, special conditions are present. At the moment of start up and shut down, in particular, strong solubility-dependent effects occur which inhibit the formation of a sufficient lubrication film, allowing the oil film to be readily washed out as a result of factors such as pressure equalization and changes in surface tension. Wear measurements on prototype compressors of different design have shown, however, that the dilution and degasification effects described can be compensated for only to some extent by using correspondingly highly viscous oils. In this respect, sufficient oil recycling from the evaporator is not always guaranteed. In addition, the higher viscosity oil leads to loss of energy efficiency and almost always a decrease in low temperature flow properties. Moreover, investigations carried out with piston compressors operated at sub-critical level have indicated that, in spite of a sufficiently high mixture viscosity, an unusually high stress is present in the area where mixed friction is present.

From a purely tribological point of view, the solubility of CO₂ in the lubricant should be as low as possible at any given temperature and pressure of operation to minimize viscosity reduction of the lubricant leading to a decrease in lubricity and load carrying ability of the lubricant/CO₂ solution. On the other hand, a satisfactory miscibility is required for oil recycling and for heat transfer in the cold cycle.

As a result, only certain chemical compounds exhibit the necessary properties to be useful as lubricants for refrigeration systems using carbon dioxide as the heat transfer agent or working fluid. Examples of such necessary properties include good low temperature flow properties, excellent lubricity and load carrying ability and miscibility with carbon dioxide over the total temperature range of operation of the equipment. As a result of the comparatively high volumetric refrigeration output of CO₂ and its increased efficiency, cryogenic compressors can be dimensioned smaller for carbon dioxide. This requires a high load carrying capacity of the lubricant in the corresponding temperature range. Investigations have shown that the physical properties and the interactions between different basic oils and sub-critical and super-critical CO₂ depend to a large extent on their chemical composition. For example, mineral oils are almost immiscible with CO₂ and exhibit only moderate high temperature stability, making them largely unsuitable for use as lubricants with CO₂-based working fluids. Because of their unfavorable phase behaviour and their comparatively low density, hydrocracked oils, alkyl aromatics and polyalphaolefins (PAO) must be classified as unsuitable for use in systems with a battery on the intake side. In addition, polyalkylene glycols have been used with carbon dioxide but cannot be used in systems having an internal motor (as for instance, in the air conditioning systems of hydrid automobiles) because of poor resistivity.

Polyol esters (POEs) are well known in the art as lubricants for displacement type refrigeration systems. Commonly used commercial POEs are derived from the reaction of a polyol (an alcohol containing 2 or more OH groups) with a monofunctional carboxylic acid. The physical characteristics of simple polyol esters are primarily derived from the structure of the acid component. Because there are a wide variety of commercially available carboxylic acids, simple polyol esters can be designed with specific physical characteristics that are optimized for a particular refrigeration system application. But for simple polyol esters there are limits to the simultaneous optimization of all desired properties. For instance, the lubricity and load carrying ability of a polyol ester lubricant is improved by using longer chain linear acids rather than shorter chain and/or branched alkyl groups. But the exact opposite may be true for miscibility with the refrigerant. So there is a careful balance required to optimize both the lubricity and load carrying ability of the lubricant with the miscibility of the lubricant and refrigerant over the widest possible temperature range of operation. In addition, the negative impact on lubricity and load carrying ability of the lubricant will become more pronounced as refrigeration system manufacturers move to lower viscosity lubricants to improve energy efficiency.

Polyol esters are especially suited for use in systems utilizing hydrofluorocarbon refrigerants (HFCs), such as R-134a and related molecules, because their polar nature provides improved miscibility with the refrigerant in comparison to other lubricants such as mineral oils, poly-alpha-olefins, or alkylated aromatics. One example of such a polyol ester lubricant is disclosed in US Patent No. 6,221,272.

Polyol esters have also been proposed for use as lubricants with CO₂-based working fluids, but to date these proposals have generally required the presence of additives to improve the high temperature properties of the ester lubricant. For example, U.S. Patent No. 7,303,693 discloses that polyalkylene glycols and/or neopentyl polyol esters, when combined with alkylated triaryl phosphate esters, are suitable for lubricating refrigerators, air-conditioning systems, heat pumps and similar systems which are operated using carbon dioxide as an operating medium. The neopentyl polyol esters are formed by reaction of neopentyl polyols, such as neopentyl glycol, pentaerythritol and trimethylol propane, with linear or branched C4 to C12 monocarboxylic acids. Preferred neopentyl polyols are said to include pentaerythritol and/or dipentaerythritol (DPE) and/or tripentaerythritol (TPE), especially mixtures comprising predominantly dipentaerythritol.

U.S. Patent No. 6,692,654 discloses a fluid composition for a refrigerating machine which comprises a refrigerating machine oil comprising a refrigerant containing carbon dioxide, an ester oil and a stabilizer in the form of a glycidyl ester epoxy compound. Suitable ester oils include esters of a diol or a polyol having 3 to 20 hydroxyl groups and a fatty acid having 6 to 20 carbon atoms. Preferred polyols are hindered alcohols such as neopentyl glycol, trimethylol ethane, trimethylol propane, trimethylol butane, di-(trimethylol propane), tri-(trimethylol propane), penthaerythritol, di-(pentaerythritol) and tri-(penthaerythritol).

However, while additives are known to assist in improving the properties of polyol esters, it is also generally accepted that their use should be minimized as they can either precipitate out from the lubricant at low temperatures (as are encountered in the evaporator) or decompose to insoluble by-products at very high temperatures (as are experienced in the compressor). Such "drop out" of the additives from the lubricant can often lead to deposits on, or complete blockage of, the refrigeration system expansion device (thermal expansion valve, capillary, or needle valve) leading to a decrease in refrigeration performance or complete failure of the system, respectively. There is also the risk that the anti-wear/extreme pressure additives (usually highly functional organic molecules containing heteroatoms) will react with the carbon dioxide refrigerant.

There is a need for an improved polyol ester lubricant for carbon dioxide-based refrigeration systems where the lubricant, preferably without the inclusion of separate additive, possesses complete miscibility with carbon dioxide over a wide temperature range of operation while also maintaining adequate lubricity and load carrying ability, provides protection against wear of refrigeration components and in addition improves the energy efficiency of the refrigeration system as compared to working fluids containing existing polyol ester lubricants.

According to the present invention, it has now been found that certain poly(neopentyl polyol) esters produced as described in U.S. Patent Nos. 3,670,013 and 5,895,778 exhibit a unique combination of improved low temperature flow properties and improved high temperature dynamic viscosity when used as lubricants with carbon dioxide-based working fluids. The poly(neopentyl polyol) esters also exhibit good miscibility with carbon dioxide over the total temperature range of operation of typical carbon dioxide refrigeration systems. Neither of U.S. Patent Nos. 3,670,013 and 5,895,778 disclose or suggest the use of these esters with carbon dioxide refrigerants.

EP-A0992572 discloses a refrigerating machine oil which comprises an ester oil, for use with a refrigerant containing carbon dioxide. US2003/0199401 discloses a refrigerator oil composition for compression refrigerators with carbon dioxide a refrigerant. EP-A2128229 discloses a refrigerating machine oil comprising an ester of a polyhydric alcohol and a fatty acid, for use with a fluoropropene or trifluoroiodomethane refrigerant. US6,267,907 discloses a lubricant-refrigerant system comprising carbon dioxide refrigerant and an aliphatic naphthalene lubricant.

### SUMMARY

In one aspect, the invention resides in a working fluid comprising (a) a refrigerant comprising carbon dioxide and (b) a polyol ester composition comprising:
(i) 45 to 55 wt% of an ester of monopentaerythritol with at least one monocarboxylic acid having 2 to 15 carbon atoms;
(ii) less than 13 wt% of an ester of dipentaerythritol with at least one monocarboxylic acid having 2 to 15 carbon atoms;
(iii) less than 10 wt% of an ester of tripentaerythritol with at least one monocarboxylic acid having 2 to 15 carbon atoms; and
(iv) at least 25 wt% of an ester of tetrapentaerythritol and higher pentaerythritol oligomers with at least one monocarboxylic acid having 2 to 15 carbon atoms;
wherein the polyol ester composition is present in a ratio of 1 to 500 parts by weight per 100 parts by weight of the refrigerant.

Conveniently, said at least one monocarboxylic acid has 5 to 11 carbon atoms, such as 6 to 10 carbon atoms. Generally, said at least one monocarboxylic acid comprises at least one linear monocarboxylic acid, such as n-pentanoic, n-heptanoic acid, n-octanoic, n-nonanoic, n-decanoic, or a mixture thereof. In one embodiment, said at least one monocarboxylic acid comprises between 15 and 100 mole percent heptanoic acid and between 85 and 0 mole percent of n-octanoic acid and/or n-decanoic acid.

### BRIEF DESCRIPTION OF THE DRAWINGS

Figure 1 is a Daniel Plot (graph of kinematic viscosity against temperature) for a working fluid comprising carbon dioxide and the polyol ester of Example 1.
Figure 2 is a Daniel Plot for a working fluid comprising carbon dioxide and the polyol ester of Example 2.
Figure 3 is a graph of kinematic viscosity at 0°C against carbon dioxide concentration for carbon dioxide working fluids comprising (a) the polyol ester of Example 1 and (b) the polyol ester of Example 2.
Figure 4 is a graph of kinematic viscosity at 100°C against carbon dioxide concentration for carbon dioxide working fluids comprising (a) the polyol ester of Example 1 and (b) the polyol ester of Example 2.

### DETAILED DESCRIPTION OF THE EMBODIMENTS

Described herein is a working fluid for a refrigeration and/or an air conditioning system wherein the working fluid employs carbon dioxide as a refrigerant and a polyol ester composition as a lubricant. The ester composition may be produced by reacting pentaerythritol with at least one monocarboxylic acid having 2 to 15 carbon atoms in a multi-stage process such that there is molar excess of hydroxyl groups in a first acid-catalyzed esterification stage and additional monocarboxylic acid is added to a second stage to complete the esterification process. The resultant ester composition is found to be soluble in the refrigerant over a broad temperature range to produce a working fluid having excellent low temperature flow properties and high temperature dynamic viscosity.

In some embodiments, pentaerythritol neopentylpolyol is used alone to produce the ester lubricant, whereas in other embodiments two or more neopentylpolyols are employed. For example, one commercially available grade of pentaerythritol contains small amounts of dipentaerythritol, tripentaerythritol, and possibly tetrapentaerythritol.

### Monocarboxylic Acid

The at least one monocarboxylic acid employed to produce the polyol ester composition has from 2 to 15 carbon atoms for example from 5 to 11 carbon atoms, such as from 6 to 10 carbon atoms. Typically the acid obeys the general formula:

R¹C(O)OH

wherein R¹ is a C₁ to C₁₂ alkyl, aryl, aralkyl or alkaryl group, such as a C₄ to C₁₀ alkyl group, for example C₅ to C₉ alkyl group. The alkyl chain R¹ may be branched or linear depending on the requirements for viscosity, viscosity index and degree of miscibility of the resulting lubricant with the refrigerant. In practice it is possible to use blends of different monobasic acids to achieve the optimum properties in the final lubricant.

Examples of suitable monocarboxylic acids include saturated, linear monocarboxylic acids including acetic acid and propionic acid, especially C₄ to C₁₀ linear monocarboxylic acids, such as butanoic acid, pentanoic acid, hexanoic acid, heptanoic acid, octanoic acid, nonanoic acid, decanoic acid and mixtures thereof; saturated, branched monocarboxylic acids, especially C₅ to C₁₀ branched monocarboxylic acids, such as the branched C5 acids (3-methylbutanoic acid and 2-methylbutanoic acid), the branched C7 acids (such as 2,4-dimethylpentanoic acid), the branched C8 acids (such as 2-ethylhexanoic acid), and the branched C9 acids (such as 3,3,5-trimethylhexanoic acid); as well as aromatic monocarboxylic acids, such as benzoic acid. Preferred monocarboxylic acids include linear monocarboxylic acids, such as n-pentanoic, n-heptanoic acid, n-octanoic, n-nonanoic, n-decanoic, and mixtures thereof.

In one embodiment, the monocarboxylic acid is n-heptanoic acid or a mixture of n-heptanoic acid with a further linear monocarboxylic acid, especially n-octanoic acid and/or n-decanoic acid. Such an acid mixture typically contains between 15 and 100 mole percent heptanoic acid and between 85 and 0 mole percent of the further linear monocarboxylic acid. In a preferred embodiment, the mixture comprises between 75 and 100 mole percent heptanoic acid and between 25 and 0 mole percent of a 3:2 molar mixture of octanoic and decanoic acids.

### Production of the Poly(Neopentylpolyol) Ester Composition

The polyol ester composition employed in the present working fluid is formed by a two step process, as described in U.S. Patent Nos. 3,670,013 and 5,895,778.

In the first step, pentaerythritol and a C₂ to C₁₅ monocarboxylic acid or acid mixture are charged to a reaction vessel such that the mole ratio of carboxyl groups to hydroxyl groups is less than 1:1, and typically is from about 1:4 to about 1:2. Also charged to the reaction vessel is at least one acid catalyst, which typically is a strong acid catalyst, that is an acid having a pKa less than 1. Examples of suitable acid catalysts include mineral acids, preferably, sulfuric acid, hydrochloric acid, and the like, acid salts such as, for example, sodium bisulfate, sodium bisulfite, and the like, sulfonic acids such as, for example, benzenesulfonic acid, toluenesulfonic acid, polystyrene sulfonic acid, methylsulfonic acid, ethylsulfonic acid, and the like.

The reaction mixture is then heated to a temperature of between about 150°C and about 250°C, typically between about 170°C and about 200°C, while acid vapor and water vapor are continuously removed from the reaction vessel, generally by the application of a vacuum source. The carboxylic acid, but not the water, removed during this step of the reaction is returned to the reactor and the reaction is continued until the desired quantity of water is removed from the reaction mixture. This can be determined by experimentation or may be estimated by calculating the expected amount of water of reaction. At this point, the mixture includes partial esters of pentaerythritol, dipentaerythritol, tripentaerythritol, tetrapentaerythritol and higher oligomeric/polymeric polyneopentylpolyols. Optionally, the acid catalyst may be neutralized with alkali at the end of the first reaction stage.

In order to complete the esterification of the partial esters, an excess of a C₂ to C₁₅ monocarboxylic acid or acid mixture acid or acid mixture and optionally an esterification catalyst is added to the reaction mixture. The additional acid can be the same or a different C₂ to C₁₅ monocarboxylic acid or acid mixture used in the initial step and is generally added in amount to provide a 10 to 25 percent excess of carboxyl groups, with respect to hydroxyl groups. The reaction mixture is then reheated to a temperature of between about 200°C and about 260°C, typically between about 230°C and about 245°C, with water of reaction removed being removed from the reaction vessel and acid being returned to the reactor. The use of vacuum will facilitate the reaction. When the hydroxyl value is reduced to a sufficiently low level, typically less than 1.0 mg KOH/g, the bulk of the excess acid is removed by vacuum distillation. Any residual acidity is neutralized with an alkali and the resulting polyol ester is recovered and dried.

The resultant ester may be used without further purification or may be purified using conventional techniques such as distillation, treatment with acid scavengers to remove trace acidity, treatment with moisture scavengers to remove moisture and/or filtration to improve clarity.

### Composition and Properties of the Polyester

The composition of the polyol ester will depend on the particular monocarboxylic acid employed to produce the ester but, the ester will have the following composition:
(i) 45 to 55 wt% of an ester of monopentaerythritol with at least one monocarboxylic acid having 2 to 15 carbon atoms;
(ii) less than 13 wt% of an ester of dipentaerythritol with at least one monocarboxylic acid having 2 to 15 carbon atoms;
(iii) less than 10 wt% of an ester of tripentaerythritol with at least one monocarboxylic acid having 2 to 15 carbon atoms; and
(iv) at least 25 wt% of an ester of tetrapentaerythritol and higher pentaerythritol oligomers with at least one monocarboxylic acid having 2 to 15 carbon atoms.

The polyol esters produced herein exhibit an advantageous combination of high viscosity index, excellent miscibility with a carbon dioxide refrigerant over a broad temperature range of about -10°C to about 120°C, and good wear resistance and load-carrying ability.

### Working Fluid

The present polyol esters are particularly intended for use as lubricants in working fluids for refrigeration and air conditioning systems, wherein the heat transfer fluid is carbon dioxide, either alone or in admixture with a hydrocarbon, a hydrofluorocarbon and/or a fluorocarbon.

The hydrocarbon refrigerants may be those which are gaseous at 25° C and one atmospheric pressure. Specific examples of the hydrocarbon refrigerants are alkanes, cycloalkanes and alkenes each having 1 to 5 carbon atoms, preferably 1 to 4 carbon atoms, such as methane, ethylene, ethane, propylene, propane, cyclopropane, butane, isobutane, cyclobutane, methylcyclopropane and a mixture of at least two kinds thereof

Non-limiting examples of suitable fluorocarbon and hydrofluorocarbon compounds include carbon tetrafluoride (R-14), difluoromethane (R-32), 1,1,1,2-tetrafluoroethane (R-134a), 1,1,2,2-tetrafluoroethane (R-134), pentafluoroethane (R-125), 1,1,1-trifluoroethane (R-143a) and tetrafluoropropene (R-1234yf). Non-limiting examples of mixtures of hydrofluorocarbons, fluorocarbons, and/or hydrocarbons include R-404A (a mixture of 1,1,1-trifluoroethane, 1,1,1,2-tetrafluoroethane and pentafluoroethane), R-410A (a mixture of 50 wt% difluoromethane and 50 wt% pentafluoroethane), R-410B (a mixture of 45 wt% difluoromethane and 55 wt% pentafluoroethane), R-417A (a mixture of 1,1,1,2-tetrafluoroethane, pentafluoroethane and n-butane), R-422D (a mixture of 1,1,1,2-tetrafluoroethane, pentafluoroethane and iso-butane), R-427A (a mixture of difluoromethane, pentafluoroethane, 1,1,1-trifluoroethane and 1,1,1,2-tetrafluoroethane) and R-507 (a mixture of pentafluoroethane and 1,1,1-trifluoroethane).

The blending ratio of carbon dioxide to hydrocarbon/ hydrofluorocarbon and/or fluorocarbon refrigerant is not particularly restricted. The total amount of hydrocarbon/ hydrofluorocarbon and/or fluorocarbon may be within the range of preferably 1 to 200 parts by weight, more preferably 10 to 100 parts by weight per 100 parts by weight of carbon dioxide.

The mixing ratio of the polyol ester lubricant to the refrigerant is also not particularly restricted. The lubricant is present in a ratio of 1 to 500 parts by weight, more preferably 2 to 400 parts by weight, per 100 parts by weight of the refrigerant.

A working fluid containing the polyol ester described above as the base oil may further contain mineral oils and/or synthetic oils such as poly-α-olefins, alkylbenzenes, esters other than those described above, polyethers, polyvinyl ethers, perfluoropolyethers, phosphoric acid esters and/or mixtures thereof.

In addition, it is possible to add to the working fluid conventional lubricant additives, such as antioxidants, extreme-pressure additives, antiwear additives, friction reducing additives, defoaming agents, profoaming agents, metal deactivators, acid scavengers and the like.

Examples of the antioxidants that can be used include phenolic antioxidants such as 2,6-di-t-butyl-4-methylphenol and 4,4'-methylenebis(2,6-di-t-butylphenol); amine antioxidants such as p,p-dioctylphenylamine, monooctyldiphenylamine, phenothiazine, 3,7-dioctylphenothiazine, phenyl-1-naphthylamine, phenyl-2-naphthylamine, alkylphenyl-1-naphthylamine, and alkylphenyl-2 -naphthylamine; sulfur-containing antioxidants such as alkyl disulfide, thiodipropionic acid esters and benzothiazole; and zinc dialkyl dithiophosphate and zinc diaryl dithiophosphate.

Examples of the extreme-pressure additives, antiwear additives, friction reducing additives that can be used include zinc compounds such as zinc dialkyl dithiophosphate and zinc diaryl dithiophosphate; sulfur compounds such as thiodipropinoic acid esters, dialkyl sulfide, dibenzyl sulfide, dialkyl polysulfide, alkylmercaptan, dibenzothiophene and 2,2'-dithiobis(benzothiazole); sulfur/nitrogen ashless antiwear additives such as dialkyldimercaptothiadiazoles and methylenebis(N,N-dialkyldithiocarbamates); phosphorus compounds such as triaryl phosphates such as tricresyl phosphate and trialkyl phosphates; dialkyl or diaryl phosphates; trialkyl or triaryl phosphites; amine salts of alkyl and dialkylphosphoric acid esters such as the dodecylamine salt of dimethylphosphoric acid ester; dialkyl or diaryl phosphites; monoalkyl or monoaryl phosphites; fluorine compounds such as perfluoroalkyl polyethers, trifluorochloroethylene polymers and graphite fluoride; silicon compounds such as a fatty acid-modified silicone; molybdenum disulfide, graphite, and the like. Examples of organic friction modifiers include long chain fatty amines and glycerol esters.

Examples of the defoaming and profoaming agents that can be used include silicone oils such as dimethylpolysiloxane and organosilicates such as diethyl silicate. Examples of the metal deactivators that can be used include benzotriazole, tolyltriazole, alizarin, quinizarin and mercaptobenzothiazole. Furthermore, epoxy compounds such as phenyl glycidyl ethers, alkyl glycidyl ethers, alkylglycidyl esters, epoxystearic acid esters and epoxidized vegetable oil, organotin compounds and boron compounds may be added as acid scavengers or stabilizers.

Examples of moisture scavengers include trialkylorthoformates such as trimethylorthoformate and triethylorthoformate, ketals such as 1,3-dioxacyclopentane, and amino ketals such as 2,2-dialkyloxazolidines.

The working fluids comprising the present polyol esters and a refrigerant can be used in a wide variety of refrigeration and heat energy transfer applications. Non-limiting examples include all ranges of air conditioning equipment from small window air conditioners, centralized home air conditioning units to light industrial air conditioners and large industrial units for factories, office buildings, apartment buildings and warehouses. Refrigeration applications include small home appliances such as home refrigerators, freezers, water coolers, vending machines and icemakers to large scale refrigerated warehouses and ice skating rinks. Also included in industrial applications would be cascade grocery store refrigeration and freezer systems. Heat energy transfer applications include heat pumps for house hold heating and hot water heaters. Transportation related applications include automotive and truck air conditioning, refrigerated semitrailers as well as refrigerated marine and rail shipping containers.

Types of compressors useful for the above applications can be classified into two broad categories; positive displacement and dynamic compressors. Positive displacement compressors increase refrigerant vapor pressure by reducing the volume of the compression chamber through work applied to the compressor's mechanism. Positive displacement compressors include many styles of compressors currently in use, such as reciprocating, rotary (rolling piston, rotary vane, single screw, twin screw), and orbital (scroll or trochoidal). Dynamic compressors increase refrigerant vapor pressure by continuous transfer of kinetic energy from the rotating member to the vapor, followed by conversion of this energy into a pressure rise. Centrifugal compressors function based on these principles. Details of the design and function of these compressors for refrigeration applications can be found in the 2008 ASHRAE Handbook, HVAC systems and Equipment, Chapter 37; the contents of which are included in its entirety by reference.

The invention will now be more particularly described with reference to the following Examples.

In the preparative Examples, the reactor was equipped with a mechanical stirrer, thermocouple, thermoregulator, Dean Stark trap, condenser, nitrogen sparger, and vacuum source.

As used herein, the term "acid value" of a polyol ester composition refers to the amount of unreacted acid in the composition and is reported as amount in mg of potassium hydroxide required to neutralize the unreacted acid in 1 gram of the composition. The acid value is measured by ASTM D 974.

### Example 1

To a reactor as described above was charged 392 grams pentaerythritol (2.88 moles), 720 grams n-heptanoic acid (5.54 moles) and a strong acid catalyst as described by Leibfried in U.S. Patent No. 3,670,013. The initial charge has a mole ratio of carboxyl groups to hydroxyl groups of 1:2.08 and the expected water of esterification from the initial charge is 5.54 moles or about 100 grams.

The mixture was heated to a temperature of about 170°C and water of reaction was removed and collected in the trap. Vacuum was applied at temperature to obtain a reflux thereby removing the water and returning the acid collected in the trap to the reactor. The temperature was maintained at 170°C under vacuum until 125 ml of water was collected. At this point the reaction mixture consisted of partial esters of pentaerythritol, dipentaerythritol, tripentaerythritol, tetrapentaerythritol, and higher oligomer esters of pentaerythritol.

After cooling the partially esterified product to about 134°C, an additional 236.6 grams (1.82 moles) of n-heptanoic acid was added, along with 264.4 grams (2.05 moles) of a 6:4 blend of n-octanoic:n-decanoic acids and an amount of alkali sufficient to neutralize the strong acid catalyst used in the first step. Heat was then applied to raise the temperature of the reaction mixture to 240°C, whereafter the mixture was maintained at this temperature for about 8 hours. At this time a total of 173 ml water has been collected and the hydroxyl value was 6.4 mg KOH/g.

The reaction mixture was then held at 240°C for about 3 additional hours, with vacuum being applied to remove excess acid overhead. When the acid value was less than 1.0 mg KOH/g, the mixture was cooled to 80°C and residual acidity was neutralized with alkali. The viscosity at 40°C was 140 cSt (1.4x10⁻⁴ m²/s) and at 100°C was 19.6 cSt (1.96x10⁻⁵ m²/s). Approximately 275 grams of a technical pentaerythritol ester of n-heptanoic, n-octanoic acid and n-decanoic acid was added to dilute the product to a target viscosity grade of ISO 68 and the product was dried and filtered. The physical properties of the resultant product are provided in Table 1.

### Example 2 (Comparative)

Comparative Example 2 is a polyol ester based synthetic refrigeration lubricant commercially available from CPI Engineering Services under the trade name Emkarate RL 68H. The base stock of Emkarate RL 68H is an ester of monopentaerythritol with a mixture of branched and linear C₅ to C₉ carboxylic acids. The physical properties of the ester of Comparative Example 2 are provided in Table 1.

**Table 1**

| Property | Example 1 Polyneopentylpolyol | Comparative Example 2 | Method |
|---|---|---|---|
| Kinematic Viscosity @ 40°C | 68.6 (6.89x10⁻⁵ m²/s) | 65.5 (6.55x10⁻⁵ m²/s) | ASTM D-445 |
| Kinematic Viscosity @ 100°C | 10.9 (1.09x10⁻⁵ m²/s) | 9.5 (9.5x10⁻⁶ m²/s) | ASTM D-445 |
| Viscosity Index | 150 | 117 | ASTM D-2270 |
| TAN, mg KOH/g | 0.02 | 0.02 | ASTM D-664 |
| Water Content, ppm | 25 | < 40 | ASTM D-1533, Method B |
| Density @ 15.6 °C, 1bs/gal | 8.23 (0.99 kg/) | 8.12 (0.97 kg/l) | ASTM D-4052 |
| Pour Point, °C | -46 | -39 | ASTM D-97 |
| Flash Point, °C | 279 | 270 | ASTM D-92 |
| ASTM Color | < 1.0 | Not reported | ASTM D-1500 |

### Example 3

The esters of Examples 1 and 2 were compared in four different wear and load carrying bench tests as described below and the results are summarized in Table 2.

### a) ASTM D 4172 4-Ball Wear Test

This test measures the wear preventive properties of a lubricant under boundary lubrication conditions. Four ball wear tests were conducted according to ASTM method D 4172 using a Falex Variable Drive Four-Ball Wear Test Machine. In the test, four balls are arranged in an equilateral tetrahedron, with the lower three balls being clamped securely in a test cup filled with lubricant and the upper ball being held by a chuck that is motor-driven. The upper ball rotates against the fixed lower balls. Load is applied in an upward direction with a pneumatic loading system which also has an air bearing to allow free movement of the sample cup for measurement of coefficient of friction if desired. Heaters allow operation at elevated oil temperatures. The three stationary steel balls are immersed in 10 milliliters of sample to be tested, and the fourth steel ball is rotated on top of the three stationary balls in "point-to-point contact." The machine is operated for one hour at 75°C with a load of 40 kilograms and a rotational speed of 1,200 revolutions per minute. At the end of the test the average diameter of the wear scars on the three lower balls is measured and reported in millimeters.

### b) ASTM D 3233 Method A, Pin-on-Vee Block Test

This test measures the extreme pressure load carrying performance of the lubricant. A steel journal held in place by a brass shear pin is rotated against two stationary V-blocks to give a four-line contact. The test pieces and their supporting jaws are immersed in the oil sample cup for oil lubricants. The journal is driven at 250 rpm and load is applied to the V-blocks through a nutcracker action lever arm and spring gage. The load is actuated and ramped continuously during the test by means of a ratchet wheel mechanism. The load is ramped by the loading ratchet mechanism until the brass shear pin shears or the test pin breaks. The torque is reported in pounds from the gauge attached to the Falex lubricant tester.

### c) Cameron-Plint Reciprocating Wear Test

The anti-wear properties of the esters of Examples 1 and 2 were also evaluated using the Cameron-Plint TE77 High Frequency Friction Machine Tester. The specimen parts (6 mm diameter AISI 52100 steel ball of 800±20 kg/mm² hardness and hardened ground NSOH B01 gauge plate of RC 60/0.4 micron) were rinsed and then sonicated for 15 minutes with technical grade hexanes. This procedure was repeated with isopropyl alcohol. The specimens were dried with nitrogen and set into the TE77 tester. The oil bath was filled with 10 mL of sample. The test was run at a 30 Hertz frequency, 100 Newton load, 2.35 mm amplitude. The test starts with the specimens and oil at room temperature. Immediately, the temperature was ramped over 15 minutes to 50°C, where it was then held constant for 15 minutes. The temperature was then ramped over 15 minutes to 100°C, where it was held constant for 45 minutes. A third temperature ramp over 15 minutes to 150°C was followed by a final dwell at 150°C for 15 minutes. The total length of the test was 2 hours. At the end of test, the wear scar diameter on the 6 mm ball was measured using a Leica StereoZoom6^{R} Stereomicroscope and a Mitutoyo 164 series Digimatic Head. Also determined was the maximum depth of the wear scar on the plate (Wear Scar Depth, µm). This was measured using a profilimeter.

### d) ASTM D 2783 Four-Ball Extreme Pressure Test

This test is similar to the anti-wear test (a) above, but starts at room temperature and the load on the four rotating balls is constantly increased until the balls weld to each other. The quantities measured to assess performance are weld point load (kgf), scar diameter (mm at 100 kgf or 126 kgf) just before weld point, and load wear index (LWI) (average of sum of the corrected loads determined for 10 applied loads preceding the weld point, kgf). A higher LWI is an indication of better anti-wear properties.

**Table 2**

| Test | Example 1 Polyneopentyl polyol ester | Comparative Example 2 |
|---|---|---|
| ASTM D-4172 4-Ball Wear Test, average wear scar, mm | 0.88 | 0.67 |
| ASTM D-3233 Method A Falex Pin and V-block, 1bs to break | 1250 (567 Kg) | 900 (408.2 Kg) |
| Cameron-Plint Wear Test Ball scar width (plate scar depth) | 0.72 (29.2) | 0.78 (31.7) |
| ASTM D 2783 4-Ball EP Test LWI/Weld Point/Last Non-seizure Load | 53.3/160/50 | 37.8/126/40 |

### Example 4

The pressure-viscosity-temperature relationship data shown in Figure 1 for combinations of the lubricant of the invention with carbon dioxide (R-744) was generated using the equipment and method described by Seeton, C. J. and Hrnjak, P. in "Thermophysical Properties of CO2-Lubricant Mixtures and Their Affect on 2-Phase Flow in Small Channel"; presented at the International Refrigeration and Air Conditioning Conference, July 17-20, paper number R-170. Corresponding data for Comparative Example 2 in combination with carbon dioxide was also acquired and is reported in Figure 2. Select data from both experiments are reported in Table 3, Figure 3 and Figure 4.

**Table 3**

| **Conditions** | Example 1 Polyneopentyl polyol ester | Comparative Example 2 |
|---|---|---|
| **110 °C and 120 Bar (12MPa)** | | |
| % Carbon Dioxide | 17 | 19 |
| Kinematic Viscosity (cSt) | 2.0 (2.0x10⁻⁶ m²/s) | 1.4 (1.4x10⁻⁶ m²/s) |

| **110 °C and 50 Bar (5MPa)** | | |
|---|---|---|
| % Carbon Dioxide | 6.5 | 8.0 |
| Kinematic Viscosity (cSt) | 4.7 (4.7x10⁻⁶ m²/s) | 3.2 (3.2x10⁻⁶ m²/s) |

The data reported in Table 3 demonstrate that, although both lubricants are compatible with carbon dioxide, carbon dioxide has a lower steady state concentration at both 50 and 120 bar (5 and 12 MPa) in the lubricant of the invention (Example 1). This results in less viscosity dilution by carbon dioxide giving a working fluid with a higher kinematic viscosity at any given pressure and temperature combination. The higher viscosity of the working fluid results in improved lubricity and load carrying ability as compared with the working fluid containing the lubricant of Comparative Example 2.

The results reported in Figure 3 demonstrate that, as compared with the lubricant of Comparative Example 2, the lubricant of Example 1 alone has a lower kinematic viscosity at 0 °C, which is important for energy conservation during start up, but a comparable viscosity at any given concentration of carbon dioxide (i.e., there is less viscosity loss due to dilution with carbon dioxide).

The results reported in Figure 4 support the data presented in Table 3 and demonstrate that at high temperature the viscosity of the refrigerant/lubricant combination of Example 1 is always higher than that for the refrigerant/lubricant combination of Comparative Example 2. This again is important for maintenance of good lubricity and load carrying of the working fluid during high temperature operation of the compressor.

## Claims

1. A working fluid comprising (a) a refrigerant comprising carbon dioxide and (b) a polyol ester composition comprising:
(i) 45 to 55 wt% of an ester of monopentaerythritol with at least one monocarboxylic acid having 2 to 15 carbon atoms;
(ii) less than 13 wt% of an ester of dipentaerythritol with at least one monocarboxylic acid having 2 to 15 carbon atoms;
(iii) less than 10 wt% of an ester of tripentaerythritol with at least one monocarboxylic acid having 2 to 15 carbon atoms; and
(iv) at least 25 wt% of an ester of tetrapentaerythritol and higher pentaerythritol oligomers with at least one monocarboxylic acid having 2 to 15 carbon atoms;
wherein the polyol ester composition is present in a ratio of 1 to 500 parts by weight per 100 parts by weight of the refrigerant.

2. The working fluid of claim 1, wherein said at least one monocarboxylic acid has 5 to 11 carbon atoms.

3. The working fluid of claim 1, wherein said at least one monocarboxylic acid has 6 to 10 carbon atoms.

4. The working fluid of claim 1, wherein said at least one monocarboxylic acid is selected from acetic acid, propionic acid, butanoic acid, pentanoic acid, hexanoic acid, heptanoic acid, octanoic acid, nonanoic acid, decanoic acid, undecanoic acid, dodecanoic acid, tridecanoic acid, tetradecanoic acid, pentadecanoic acid, 3-methylbutanoic acid, 2-methylbutanoic acid, 2-ethylhexanoic acid, 2,4-dimethylpentanoic acid, 3,3,5-trimethylhexanoic acid, benzoic acid and mixtures thereof.

5. The working fluid of any preceding claim, wherein said at least one monocarboxylic acid comprises at least one linear monocarboxylic acid.

6. The working fluid of claim 1, wherein said at least one monocarboxylic acid is selected from n-pentanoic, n-heptanoic acid, n-octanoic, n-nonanoic, n-decanoic, and mixtures thereof.

7. The working fluid of claim 1, wherein said at least one monocarboxylic acid comprises between 15 and 100 mole percent heptanoic acid and between 85 and 0 mole percent of n-octanoic acid and/or n-decanoic acid.

8. The working fluid of any preceding claim, wherein the refrigerant further comprises at least one of a hydrocarbon, a hydrofluorocarbon and a fluorocarbon.

9. The working fluid of any of claims 1 to 7, wherein carbon dioxide is the sole refrigerant.

## Patentansprüche

1. Arbeitsfluid, umfassend (a) ein Kältemittel, das Kohlendioxid umfasst, und (b) eine Polyolesterzusammensetzung, umfassend:
(i) 45 bis 55 Gew.-% eines Esters von Monopentaerythritol mit mindestens einer Monocarbonsäure mit 2 bis 15 Kohlenstoffatomen;
(ii) weniger als 13 Gew.-% eines Esters von Dipentaerythritol mit mindestens einer Monocarbonsäure mit 2 bis 15 Kohlenstoffatomen;
(iii) weniger als 10 Gew.-% eines Esters von Tripentaerythritol mit mindestens einer Monocarbonsäure mit 2 bis 15 Kohlenstoffatomen;
(iv) mindestens 25 Gew.-% eines Esters von Tetrapentaerythritol und höheren Pentaerythritol-Oligomeren mit mindestens einer Monocarbonsäure mit 2 bis 15 Kohlenstoffatomen;
wobei die Polyolesterzusammensetzung in einem Anteil von 1 bis 500 Gewichtsteilen pro 100 Gewichtsteile des Kältemittels vorliegt.

2. Arbeitsfluid nach Anspruch 1, wobei die mindestens eine Monocarbonsäure 5 bis 11 Kohlenstoffatome aufweist.

3. Arbeitsfluid nach Anspruch 1, wobei die mindestens eine Monocarbonsäure 6 bis 10 Kohlenstoffatome aufweist.

4. Arbeitsfluid nach Anspruch 1, wobei die mindestens eine Monocarbonsäure aus Essigsäure, Propionsäure, Butansäure, Pentansäure, Hexansäure, Heptansäure, Octansäure, Nonansäure, Decansäure, Undecansäure, Dodecansäure, Tridecansäure, Tetradecansäure, Pentadecansäure, 3-Methylbutansäure, 2-Methylbutansäure, 2-Ethylhexansäure, 2,4-Dimethylpentansäure, 3,3,5-Trimethylhexansäure, Benzoesäure und Mischungen davon ausgewählt ist.

5. Arbeitsfluid nach einem der vorhergehenden Ansprüche, wobei die mindestens eine Monocarbonsäure mindestens eine lineare Monocarbonsäure umfasst.

6. Arbeitsfluid nach Anspruch 1, wobei die mindestens eine Monocarbonsäure aus n-Pentansäure, n-Heptansäure, n-Octansäure, n-Nonansäure, n-Decansäure und Mischungen davon ausgewählt ist.

7. Arbeitsfluid nach Anspruch 1, wobei die mindestens eine Monocarbonsäure zwischen 15 und 100 Molprozent Heptansäure und zwischen 85 und 0 Molprozent n-Octansäure und/oder n-Decansäure umfasst.

8. Arbeitsfluid nach einem der vorhergehenden Ansprüche, wobei das Kältemittel ferner einen Kohlenwasserstoff, einen teilfluorierten Kohlenwasserstoff und/oder einen vollfluorierten Kohlenwasserstoff umfasst.

9. Arbeitsfluid nach einem der Ansprüche 1 bis 7, wobei Kohlendioxid das einzige Kältemittel ist.

## Revendications

1. Fluide de travail comprenant (a) un réfrigérant comprenant du dioxyde de carbone et (b) une composition d'esters de polyols comprenant :
(i) 45 à 55 % en poids d'un ester de monopentaérythritol avec au moins un acide monocarboxylique ayant 2 à 15 atomes de carbone ;
(ii) moins de 13 % en poids d'un ester de dipentaérythritol avec au moins un acide monocarboxylique ayant 2 à 15 atomes de carbone ;
(iii) moins de 10 % en poids d'un ester de tripentaérythritol avec au moins un acide monocarboxylique ayant 2 à 15 atomes de carbone ; et
(iv) au moins 25 % en poids d'un ester de tétrapentaérythritol et d'oligomères de pentaérythritol supérieurs avec au moins un acide monocarboxylique ayant 2 à 15 atomes de carbone ;
la composition d'esters de polyols étant présente dans un rapport de 1 à 500 parties en poids pour 100 parties en poids du réfrigérant.

2. Fluide de travail de la revendication 1, dans lequel ledit au moins un acide monocarboxylique a 5 à 11 atomes de carbone.

3. Fluide de travail de la revendication 1, dans lequel ledit au moins un acide monocarboxylique a 6 à 10 atomes de carbone.

4. Fluide de travail de la revendication 1, dans lequel ledit au moins un acide monocarboxylique est choisi parmi l'acide acétique, l'acide propionique, l'acide butanoïque, l'acide pentanoïque, l'acide hexanoïque, l'acide heptanoïque, l'acide octanoïque, l'acide nonanoïque, l'acide décanoïque, l'acide undécanoïque, l'acide dodécanoïque, l'acide tridécanoïque, l'acide tétradécanoïque, l'acide pentadécanoïque, l'acide 3-méthylbutanoïque, l'acide 2-méthylbutanoïque, l'acide 2-éthylhexanoïque, l'acide 2,4-diméthylpentanoïque, l'acide 3,3,5-triméthylhexanoïque, l'acide benzoïque et les mélanges de ceux-ci.

5. Fluide de travail d'une quelconque revendication précédente, dans lequel ledit au moins un acide monocarboxylique comprend au moins un acide monocarboxylique linéaire.

6. Fluide de travail de la revendication 1, dans lequel ledit au moins un acide monocarboxylique est choisi parmi les acides n-pentanoïque, n-heptanoïque, n-octanoïque, n-nonanoïque, n-décanoïque, et les mélanges de ceux-ci.

7. Fluide de travail de la revendication 1, dans lequel ledit au moins un acide monocarboxylique comprend entre 15 et 100 pour cent en moles d'acide heptanoïque et entre 85 et 0 pour cent en moles d'acide n-octanoïque et/ou d'acide n-décanoïque.

8. Fluide de travail d'une quelconque revendication précédente, dans lequel le réfrigérant comprend en outre un hydrocarbure, et/ou un hydrofluorocarbure, et/ou un fluorocarbure.

9. Fluide de travail de l'une quelconque des revendications 1 à 7, dans lequel le dioxyde de carbone est l'unique réfrigérant.
